

1

2,928,713

## CHROMIC ACID TREATMENT OF FEATHERS

Varsenig Z. Pasternak and Robert M. Lollar, Cincinnati, Ohio, assignors to the United States of America as represented by the Secretary of the Army

No Drawing. Application April 23, 1957  
Serial No. 654,615

8 Claims. (Cl. 8—94.10)

This invention relates to a method of treating land fowl feathers, especially chicken feathers, to increase their "filling power" and resiliency, and to impart permanent curliness and water repellency, thereby making such feathers an acceptable substitute for the standard down and feather mixture now in wide use for sleeping bags, comforters, etc. Another object is to provide a treatment which enables the feathers to retain much of their high filling power after several washings with a detergent. A further object is to employ a chemical treatment which will make the feathers resistant to moths. Other objects will be apparent from the following description of the method presently preferred by us.

In explanation of the term "filling power," reference may be made to the report entitled "A Proposed Method for Measuring the Filling Power of Down and Feathers" by Henry A. Sinski, publication No. TD103037, The Office of Technical Services, Department of Commerce, and to the article by N. B. Edelman in Textile Research Journal, vol. 17, p. 199 (April 1947), entitled "Investigation of Methods for Determining the Filling Power of Feathers." See also the Sinski et al. Patent No. 2,706,910 dated April 26, 1955. Ordinarily, chicken feathers have a filling power of 1.8 to 2.1 cm., while the 40/60 down-feather mixture has a filling power of 5.3 to 5.9 cm.

The term "feathers" as used herein includes whole land fowl feathers of the desired size range, crushed (commercial "curled") land fowl feathers, land fowl feather fibers, stripped land fowl feathers, and mixtures of these.

In the preferred procedure, the feathers, if not known to be entirely free from blood, are first soaked for about ten minutes in a water solution of a commercial blood solubilizer, such as "Coagusol" (a mixture of sodium hexametaphosphate and alcohol sulfate). After the soaking, the solution is drained from the feathers and the feathers are then laundered or dry cleaned. In laundering, preferably a detergent such as "Tergitol NPX" (alkyl phenyl ether of polyethylene glycol) is used (0.25% water solution at 110°—125° F.). Other non-ionic detergents have been found to be satisfactory. In general, the non-ionic type of detergents should be used to obviate any action on the protein of the feathers. Laundering continues for about twenty minutes, then the solution is removed from the feathers by centrifuging or wringing. While a number of well-known dry cleaning solutions could be used to clean the feathers, laundering is preferred because it is less expensive. Both laundering and dry cleaning may take place in the same vessel or container that is used during the blood-solubilizing step. Of course, if the feathers as initially received are perfectly clean, the soaking and washing or dry cleaning may be omitted.

If the feathers are from immature chickens, the damp feathers from the described laundering or dry cleaning operation are placed in a 1% water solution of trisodium phosphate  $Na_3PO_4 \cdot 12H_2O$  at 43°—49° C. for about ten minutes. If feathers from mature chickens are being processed, the phosphate treatment period is increased to

2

about thirty minutes. This mild alkaline treatment of the feathers is believed to alter the stability of the feathers by modification of the cystine linkages in the keratin. This step is important because it materially increases the curliness of the feathers, and it curls naturally uncurl mature feathers, thereby increasing the bulk value of the final feather product. Other suitably buffered alkaline solutions, for example, sodium carbonate or borax, may be used in lieu of the phosphate solution mentioned above, but in all cases the time of the treatment must be less for immature feathers to avoid excessive degradation. Trisodium phosphate is preferred because of its quicker action due to a higher pH. It is believed that the higher concentration of cystine linkages in mature feathers enables them to resist the action of the alkaline solution for a longer period.

The data from successful laboratory runs at The Tanners' Council Research Laboratory, University of Cincinnati will now be given.

### Bromoacetic acid—Chromic acid—Hydrazine treatment

A bath of 45 grams of chicken feathers was first treated with trisodium phosphate as described above. The feathers were removed from the bath and thoroughly rinsed with water, then they were treated with a 5% bromoacetic acid solution (56 g. bromoacetic acid in 900 ml. water) which was neutralized to pH 7 by the addition of 90 ml. of 10%  $Na_2CO_3$  solution. After fifteen minutes, the pH was raised to 9—9.5 and the feathers were kept in the bath for 4½ hours at 48°—51° C. Then the feathers were removed and thoroughly rinsed. Next the feathers were placed in a chromic acid bath (1000 ml. of 0.8% chromic acid or 1% sodium bichromate of pH 2.5—2.7) and kept there for 2½ hours at 34°—44° C. Then the feathers were transferred to a bath of 1000 ml. of 0.1% hydrazine solution and kept there at 37°—31° C. for about one hour, say 63 minutes. The pH of the solution rose from about 3.0 to between 4.0 and 5.0. Then the pH was raised to 7 and the feathers were kept in the neutral bath for six minutes more, then were rinsed for thirty minutes and dried with agitation for forty minutes. After letting the feathers relax for eight days, the filling power was measured and found to be 6.8 cm. After twice laundering the treated feathers, the filling power was 6.4 cm.

### Chloroacetic acid+Chromic acid+Hydrazine treatment

A batch of 67 grams of chicken feathers was first given the described phosphate treatment, then was rinsed for twenty minutes. Then the feathers were put in a bath of 1500 ml. of 2.4% chloroacetic acid (monochloroacetic acid) for twenty minutes at pH 2.9 and 42° C. Next sodium carbonate solution was added to raise the pH, and the feathers were kept in the sodium chloroacetic acid solution for two hours at pH 9.2—9.4, temperature 41°—47° C. Then the feathers were well rinsed and were immersed in a chromic acid bath (15 g. sodium bichromate in 1500 ml. of water plus 2 ml. of concentrated sulfuric acid) to two hours at 41°—45° C., the pH being 2.5—2.7. The next step was to transfer the feathers to a hydrazine bath (6 g. of hydrazine sulfate plus 1300 g. of water plus 200 g. of mother liquor, which was spent chromic acid solution; i.e., chromic acid solution left over from the chromic acid bath described in the preceding sentence, after removal of the feathers therefrom). The feathers were kept in this reducing bath for fifty minutes at pH 4.2, temperature 38°—42° C. Then the pH was raised to 6.8, the temperature remaining about the same, and after ten minutes the feathers were removed, rinsed for twenty-five minutes, dried and relaxed. The filling power reading was 6.3 cm. After being laundered and

tumble-dried, the treated feathers had a filling power of 6.1 cm.

*Basic chromic sulfate treatment*

This example describes a feather treatment with a basic chromic sulfate bath. The basic chromic sulfate used in this example is "Tanolin R," which is a trade name for one-third basic chromic sulfate containing about 25% chromic oxide. The recommended procedure for employing this tanning agent for the treatment of chicken feathers is as follows.

After the described phosphate treatment, rinse the feathers to neutrality, then put the wet feathers in a solution of 1,000 ml. of 1.5% basic chromic sulfate (e.g., "Tanolin R") at pH 3.5-3.8 and 43°-46° C. for about 170 minutes. Then raise the pH to 6.0 and keep the feathers in the bath for ten minutes longer, with occasional stirring, at 44° C. Then rinse thoroughly and tumble dry at about 43° C. (black bulb temperature) the temperature rising to 110° C. when the feathers are dry. The filling power is 6.0 cm.

Another procedure giving about the same results is as follows: After the phosphate treatment, a 67 gram bath of chicken feathers is well rinsed and then put in a 3.5% bath of bromoacetic acid solution at pH 2.9, the temperature being 42° C. After fifteen minutes, the pH of the solution is raised to 9.5 and the feathers are kept in the solution for about two hours at 41°-47° C. Then the feathers are rinsed again and treated for three hours with basic chromic sulfate (e.g., "Tanolin R") at 42°-46° C., the pH being 4.1-3.8. Finally, the pH of the solution is raised to 6.4, and the feathers are kept in the sludge for fifteen minutes longer. Finally, the feathers are rinsed for twenty minutes, dried, and relaxed. The filling power is 6.0 cm.

*Two bath chromic acid treatment*

A batch of 67 grams of chicken feathers was given the phosphate treatment already described, then the feathers were carefully rinsed. The damp feathers were put in a chromic acid bath (1500 ml. of 1% sodium bichromate solution or 0.8% chromic acid) for two and one-half hours at 39°-43° C. and pH 28.5-2.7. Then the feathers were put in a hydrazine bath (6 g. of hydrazine sulfate plus 1300 ml. of water plus 200 ml. of spent chromic acid solution) and kept there for thirty minutes at 37°-43° C., the pH being 3.9-4.0. Then the pH was raised to 7.1 and the feathers were kept in the sludge for ten minutes longer. After this, they were rinsed, dried, and relaxed. The filling power was 6.3 cm. After laundering, drying and relaxing, the filling power rose to 6.6 cm. Evidently the two-bath chrome treatment caused more deep-seated and permanent changes in the feathers than the one-bath treatment previously described.

Obviously the invention is not limited to the details described in the foregoing, but is defined in the appended claims.

*What we claim is:*

1. A method of treating land fowl feathers to enhance their filling power, which comprises modifying the cystine linkage of the keratin of said land fowl feathers by soaking said feathers in an aqueous alkaline solution until their curliness is increased, rinsing said feathers, then placing said land fowl feathers for at least about 2 hours in an aqueous bath containing dissolved therein a chromium compound being a member of the group consisting of chromic acid and a basic chromic sulfate at about 34°-46° C., the initial pH of said bath being about 2.5-2.7 when said dissolved chromium compound is chromic acid and about 3.5-4.1 when said dissolved chromium compound is a basic chromic sulfate; then continuing the immersion of said feathers in an aqueous bath having a pH of about 6-7, said aqueous bath containing dissolved therein a member of the group consisting of chromic acid, a basic chromic sulfate,

hydrazine, and a mixture of hydrazine sulfate and spent chromic acid, the total time of immersion of said feathers being sufficient to increase substantially the filling power of said feathers, then removing said feathers and rinsing and drying them.

2. The method according to claim 1, wherein said aqueous alkaline solution is an approximately 1% solution of trisodium phosphate having a temperature of about 43°-49° C., said soaking having a duration of about 10-30 minutes.

3. A method of treating land fowl feathers to enhance their filling power, which comprises modifying the cystine linkage of the keratin of said land fowl feathers by soaking said feathers in an aqueous alkaline solution until their curliness is increased, rinsing said feathers, then placing said feathers in about 5% bromoacetic acid aqueous solution neutralized to about pH 7, then after about fifteen minutes raising the pH to about 9-9.5, the feathers being kept in the bath for about 4½ hours at about 48°-51° C.; then rinsing the feathers and placing them in an aqueous chromic acid bath for about 2½ hours at about 34°-44° C. and a pH of about 2.5-2.7; then transferring the feathers to an about 0.1% hydrazine aqueous solution and keeping them in said solution for about one hour at about 37°-31° C.; then raising the pH to about 7, removing said feathers from the bath after their filling power has been substantially increased, then rinsing and drying them.

4. A method of treating land fowl feathers to enhance their filling power, which comprises modifying the cystine linkage of the keratin of said land fowl feathers by soaking said feathers in an aqueous alkaline solution until their curliness is increased, rinsing said feathers, then placing the land fowl feathers in an about 2.4% chloroacetic acid solution for about 20 minutes at a pH of about 2.9 and about 42° C.; then raising the pH to about 9.2-9.4 and keeping the feathers in the alkaline bath at about 41°-47° C. for about 2 hours; then rinsing the feathers; then putting the feathers in a chromic acid bath made from about 15 g. sodium bichromate in about 1500 ml. of water and about 2 ml. of concentrated sulfuric acid, at about 41°-45° C. and a pH of about 2.5-2.7 for about 2 hours; then transferring the feathers to a hydrazine aqueous solution at pH about 4.2 and a temperature of about 38°-42° C. for about fifty minutes, raising the pH to about 6.8 for about ten minutes, then rinsing the feathers and drying them.

5. A method of treating land fowl feathers to enhance their filling power, which comprises modifying the cystine linkage of the keratin of said land fowl feathers by soaking said feathers in an aqueous alkaline solution until their curliness is increased, rinsing said feathers, then placing the land fowl feathers in an about 0.8% chromic acid aqueous solution for about 2½ hours at about 39°-43° C. and a pH of about 2.5-2.7; then putting the feathers in an aqueous hydrazine bath in the presence of spent chromic acid dissolved in said bath; keeping the feathers in said bath at about 37°-43° C. for about thirty minutes, the pH being about 3.9 to 4.0, then raising the pH to about 7 and keeping the feathers in the substantially neutral solution for about 10 minutes, then removing the feathers from said solution and rinsing and drying them.

6. A method of treating land fowl feathers to enhance their filling power, which comprises modifying the cystine linkage of the keratin of said land fowl feathers by soaking said feathers in an aqueous alkaline solution until their curliness is increased, rinsing said feathers, then putting the land fowl feathers in an about 1.5% aqueous solution of a basic chromic sulfate at a pH of about 3.5-3.8 and a temperature of 43°-46° C. for about 170 minutes, then raising the pH to about 6.0 and keeping the feathers in the bath at about 44° C. for about ten additional minutes, then rinsing and drying them.

7. A method of treating land fowl feathers to enhance

their filling power, which comprises modifying the cystine linkage of the keratin of said land fowl feathers by soaking said feathers in an aqueous alkaline solution until their curliness is increased, rinsing said feathers, then placing said feathers in an about 3.5% bromoacetic acid aqueous solution at a pH of about 2.9, then after about 15 minutes raising the pH to about 9.5, keeping said feathers in said solution for about 2 hours at about 41°-47° C.; then rinsing the feathers and placing them in an aqueous solution of a basic chromic sulfate at a pH of about 10 3.8-4.1 and a temperature of about 42°-46° C. for about 3 hours, then raising the pH to about 6.4 and keeping the feathers in said chromic acid solution for about 15 additional minutes, then rinsing said feathers and drying them.

8. The product produced by the method of claim 1.

References Cited in the file of this patent

UNITED STATES PATENTS

|           |           |                |
|-----------|-----------|----------------|
| 625,345   | Millar    | May 23, 1899   |
| 2,184,147 | Lowe      | Dec. 19, 1939  |
| 2,261,094 | Speakman  | Oct. 28, 1941  |
| 2,426,861 | Comolli   | Sept. 2, 1947  |
| 2,805,913 | Frederick | Sept. 2, 1957  |
| 2,805,914 | Frederick | Sept. 10, 1957 |

OTHER REFERENCES

Speakman: Jour. of the Soc. of Dyers and Colourists, September 1936, pp. 335-346.

15 Speakman: Jour. of the Soc. of Dyers and Colourists, June 1937, pp. 236-242.